

Patented Feb. 1, 1927.

1,616,352

# UNITED STATES PATENT OFFICE.

ERNEST B. COBB, OF JERSEY CITY, NEW JERSEY, ASSIGNOR TO STANDARD DEVELOPMENT COMPANY, A CORPORATION OF DELAWARE.

## MANUFACTURE OF REFINED OILS.

No Drawing.

Application filed April 8, 1922. Serial No. 550,865.

The present invention relates to the manufacture of refined oils and more particularly of refined viscous oils such as lubricating oils, water white or medicinal oils and the like.

In the refining of such oils, the stock, which is in general a distillate or cut obtained from crude oil after the kerosene or burning oil cut has been removed, is subjected to an acid treatment with strong sulfuric acid, for example, with 66° Bé. acid or fuming acid. The treatment with sulfuric acid may be heavy or light; that is, with greater or less amounts of acid, in accordance with the extent to which the refining of the oil is to be carried. The action of the acid upon the hydrocarbons of the oil appears to form, among other compounds, sulfo-compounds which are in part dissolved in the sludge which is settled out of the oil, and are in part retained in the oil. The sulfo-compounds retained in the oil, both in their acid state and when neutralized, appear to act as emulsifying agents, causing the oil to readily form persistent emulsions when washed with water. In the case of water white and medicinal oils they likewise tend to discolor the oil and to make it unsuitable for internal administration. The removal of these sulfo-compounds or emulsion inducing constituents substantially removes the tendency of the treated oil to emulsify.

The proportion and the specific characteristics of the sulfo-compounds retained in the oil vary to some extent with the character of oil treated and with the nature of the treatment. Thus, in a light acid treatment with 66° Bé. acid for the production of lubricating oils, a less proportion of these compounds appears to be formed than in the heavy acid treatments with fuming acid employed in the case of the manufacture of white oils or medicinal oils. The character of the oil appears to influence to a marked degree the ease of removal of the retained sulfo-compounds. Thus it has been found that Russian oil distillates are more amenable to the purifying treatment hereinafter set forth than distillates from coastal oils and from paraffin bearing oils such as Pennsylvania or Mid-Continent oils. Thus, although Russian oils subjected to a heavy fuming acid treatment may be directly purified by the present process, the other oils,

particularly those of 150 seconds viscosity or higher, can best be purified by such treatment after a lighter acid treatment or after a retreatment following a previous acid treatment and removal of sulfo-compounds. 60

In accordance with the present invention, the oil to be refined is subjected to the desired acid treatment which may be with 66° Baumé acid or fuming acid and in one or a plurality of dumps. The sludge is removed 65 from the treated oil as completely as possible by settling, and, if equipment permits, it is desirable that this settling be continued for two or three days or even longer. The separated oil is then heated to a temperature between 350 and 500° F., and preferably at about 380° F. for a period of fifteen hours or longer. Twenty hours has been found most suitable. During this heating it is found that the sulfo-compounds 70 tend to break down, with the formation of some volatile and some non-volatile products. In order to carry off the volatile products formed, it is found desirable to pass steam through the oil during the heat treatment, the steam being also effective in agitating the oil to cause uniform heating thereof and in removing any volatile oil present not desired in the final product. During the heat treatment acidity of the oil decreases, and it 75 becomes substantially neutral at the end of the treatment. The removal of the non-volatile products of decomposition of the sulfo-compounds from the oil, if they are not excessively large in amount, may be effected 80 by filtration of the oil through fuller's earth or Florida clay. When the proportion of decomposition products formed is so large or they are of such character that filtration through Florida clay alone is not wholly effective or is uneconomical, the colloidal products of decomposition may be in whole or in part removed by washing with acid, preferably sulfuric acid of 66° Bé. or weaker. After this washing, the oil having been thoroughly settled, its refining may be completed by direct filtration through fuller's earth. 85 90 95 100 105

The following examples illustrate the practice of the present invention:

### Example No. 1.

A Russian oil distillate of 300 to 325 seconds viscosity (Saybolt) at 100° F. was treated for the production of a medicinal oil 110

with fuming sulfuric acid, using 30% by volume of fuming acid containing 20% anhydride. The acid was used in five nearly equal dumps, the oil being preferably brought to a temperature of 70° F. or lower before each dump was used and being thoroughly settled for twenty-four to forty-eight hours after each dump. After the final acid dump the oil is settled as thoroughly as possible, preferably two or three days or longer. The sour oil is then introduced into fired stills and is heated to between 350 to 500° F., and preferably about 380 to 410°, for eighteen to twenty hours. During the heating steam is injected into the oil, and carries with it volatile products of decomposition of the sulfo-compounds, together with any constituents of the oil which undesirably reduce its flash point. The oil may be immediately cooled and filtered after this heat treatment; however, the proportion of unvolatilized products of decomposition present in it, in part appearing as colloid particles, renders filtration at this point uneconomical. It is preferred to treat the oil with an acid, for example, 66° Bé. sulfuric acid or lighter acid, 5 to 10% by volume being a suitable proportion. On settling, it is found that the oil has been to a considerable extent freed from the suspended colloids, which apparently go into the acid layer. After thorough settling, say from two days to a week, the oil is filtered through fuller's earth or Florida clay. The resulting oil has a viscosity of 200 to 250 seconds Saybolt at 100° F. and a flash point of 350 to 375° F.

*Example No. 2.*

In preparing a medicinal oil from West Colombia or Coastal stock, which appears to contain both naphthenic and asphaltic compounds, a suitable distillate is selected, for example one having a viscosity of 450 seconds Saybolt at 100° F., a gravity of about 22° Bé. and a flash point of 370° F. This stock is treated with fuming sulfuric acid containing 20% anhydride, a suitable proportion being 37% by volume. The treatment is preferably effected in five dumps of approximately equal proportions. After each dump the oil is settled, suitably from twenty-four to forty-eight hours and the sludge removed. Before each dump the oil is preferably cooled to below 70° F. After the last treatment, the sludge is drawn off and the batch is neutralized, for example, with 12° Bé. caustic soda solution. The alkali sludge is removed and the oil may then, if desired, be blown with air at about 180 to 200° F. This air blowing removes water. After neutralization the oil is distilled with fire and steam to a bottom of 5 to 10%, the distillate fraction (90-95%) being collected as a whole with the exception of the light constituents which might unde-

sirably reduce the flash point of the product. This distillation, as described in my Patent No. 1,388,517, granted August 23, 1921, leaves the sulfo-compounds in the form of their sodium salts or soaps in the residue, the 70 distillate being substantially free therefrom.

The distillate may be chilled or pressed to remove wax, if desired, and is treated again with a small proportion of the fuming acid. A suitable proportion is 15% by volume, the 75 treatment being preferably carried out in two dumps of approximately equal proportions. After this acid treatment the oil is allowed to settle for as long a period as possible, two or three days at least. The sour oil is then subjected to the heat treatment above described, being heated preferably to 380 to 410° F. for about twenty hours, with the injection of steam to effect the removal of volatile decomposition products and sulphur dioxide. At the end of the heat treatment the oil is cooled and filtered through fuller's earth, the preliminary coagulation of suspended matter with acid as described in the first example being desirable but not 90 usually necessary in this case. The finished oil has a viscosity of 200 to 210 seconds Saybolt at 100° and a gravity of about 29° Bé.

*Example No. 3.*

A distillate from a Coastal crude having a gravity of 22.3° Bé., a flash point of 325° F., a viscosity of 125 seconds Saybolt at 100° F. and a zero cold test is treated for the production of a white medicinal oil in 100 the manner described in Example No. 2, above, except that the pressing of the distillate from the oil after the first acid treatment is unnecessary and the heat treatment or steaming of the oil after the second acid 105 treatment is carried out at about 380° F. The finished oil is water white, and has a gravity of 29.8° Bé., a flash point of 325° F., a viscosity of 105 seconds Saybolt at 100° F. and a 10° F. cold test. A distillate 110 of this character may likewise be treated in the same manner as the Russian oil distillate in Example 1, a vigorous treatment with fuming acid being followed by a heat treatment in the manner described for the removal 115 of sulfo-compounds, and this, in turn, by a light acid treatment and filtration.

Although the present invention has been described in connection with the details of specific methods for carrying it into effect, 120 it is not intended that these shall be regarded as limitations upon the scope of the invention, except in so far as retained in the accompanying claims.

I claim:

1. The process of destroying emulsion inducing compounds including sulfo-compounds present in sulfuric acid treated oils by reason of the acid treatment thereof which comprises maintaining such oils at a 130

- temperature of 350 to 500° F. until decomposition of such emulsion inducing compounds including sulfo-compounds is effected within the oil body.
5. 2. The process of destroying emulsion inducing compounds including sulfo-compounds present in sulfuric acid treated oils by reason of the acid treatment thereof which comprises maintaining such oils at a 10 temperature of 350 to 500° F. until decomposition of such emulsion inducing compounds including sulfo-compounds is effected within the oil body and removing products of decomposition from the oil.
15. 3. The process of destroying emulsion inducing compounds including sulfo-compounds present in sulfuric acid treated oils by reason of the acid treatment thereof which comprises maintaining such oils at a 20 temperature of 350 to 500° F. until decomposition of such emulsion inducing compounds including sulfo-compounds is effected within the oil body, and subsequently filtering the oil.
25. 4. The process of destroying emulsion inducing compounds including sulfo-compounds present in sulfuric acid treated oils by reason of the acid treatment thereof which comprises maintaining such oils at a 30 temperature of 350 to 500° F. until decomposition of such emulsion inducing compounds including sulfo-compounds is effected within the oil body and passing steam through the oil during the heat treatment thereof.
35. 5. The process of destroying emulsion inducing compounds including sulfo-compounds present in sulfuric acid treated oils by reason of the acid treatment thereof which comprises maintaining such oils at a 40 temperature of 350 to 500° F. until decomposition of such emulsion inducing compounds including sulfo-compounds is effected within the oil body, passing steam through the oil during the heat treatment, and subsequently filtering the oil.
45. 6. The process of destroying emulsion inducing compounds including sulfo-compounds present in sulfuric acid treated oils by reason of the acid treatment thereof which comprises maintaining such oils at a 50 temperature of 350 to 500° F. until decomposition of such emulsion inducing compounds including sulfo-compounds is effected within the oil body, and washing the oil with an acid solution.
55. 7. The process of destroying emulsion inducing compounds including sulfo-compounds present in sulfuric acid treated oils by reason of the acid treatment thereof which comprises maintaining such oils at a 60 temperature of 350 to 500° F. until decomposition of such emulsion inducing compounds including sulfo-compounds is effected within the oil body, washing the oil with an acid solution, separating and filtering the oil.
8. The process of destroying emulsion inducing compounds including sulfo-compounds present in sulfuric acid treated oils 70 by reason of the acid treatment thereof which comprises maintaining such oils at a temperature of 350 to 500° F. until decomposition of such emulsion inducing compounds including sulfo-compounds is effected within the oil body, passing steam through the oil during such treatment and washing the treated oil with an acid solution.
9. The process of destroying emulsion inducing compounds including sulfo-compounds present in sulfuric acid treated oils 80 by reason of the acid treatment thereof which comprises maintaining such oils at a temperature of 350 to 500° F. until decomposition of such emulsion inducing compounds including sulfo-compounds is effected within the oil body, passing steam through the oil during the heat treatment, washing the treated oil with an acid solution, separating and filtering the oil. 85
10. The process of destroying emulsion inducing compounds including sulfo-compounds present in sulfuric acid treated oils by reason of the acid treatment thereof which comprises maintaining such oils at 90 380 to 410° F. for eighteen to twenty hours.
11. The process of destroying emulsion inducing compounds including sulfo-compounds present in sulfuric acid treated oils by reason of the acid treatment thereof 95 which comprises maintaining such oils at 380 to 410° F. for eighteen to twenty hours and removing products of decomposition from the oil.
12. The process of destroying emulsion inducing compounds including sulfo-compounds present in sulfuric acid treated oils by reason of the acid treatment thereof which comprises maintaining such oils at 100 380 to 410° F. for eighteen to twenty hours and subsequently filtering the oil. 105
13. The process of destroying emulsion inducing compounds including sulfo-compounds present in sulfuric acid treated oils by reason of the acid treatment thereof 110 which comprises maintaining such oils at 380 to 410° F. for eighteen to twenty hours and passing steam through the oil during the heat treatment thereof.
14. The process of destroying emulsion inducing compounds including sulfo-compounds present in sulfuric acid treated oils by reason of the acid treatment thereof which comprises maintaining such oils at 115 380 to 410° F. for eighteen to twenty hours, passing steam through the oil during the heat treatment, and subsequently filtering the oil. 120
15. The process of destroying emulsion inducing compounds including sulfo-compounds present in sulfuric acid treated oils 125

by reason of the acid treatment thereof which comprises maintaining such oils at 380 to 410° F. for eighteen to twenty hours, and washing the oil with an acid solution.

5. 16. The process of destroying emulsion inducing compounds including sulfo-compounds present in sulfuric acid treated oils by reason of the acid treatment thereof which comprises maintaining such oils at 380 to 410° F. for eighteen to twenty hours, 10 washing the oil with an acid solution, separating and filtering the oil.

17. The process of destroying emulsion inducing compounds including sulfo-compounds present in sulfuric acid treated oils by reason of the acid treatment thereof which comprises maintaining such oils at 380 to 410° F. for eighteen to twenty hours, 15 passing steam through the oil during such treatment and washing the treated oil with an acid solution.

18. The process of destroying emulsion inducing compounds including sulfo-compounds present in sulfuric acid treated oils by reason of the acid treatment thereof which comprises maintaining such oils at 380 20 to 410° F. for eighteen to twenty hours, 25 passing steam through the oil during such treatment and washing the treated oil with an acid solution.

to 410° F. for eighteen to twenty hours, passing steam through the oil during the heat treatment, washing the treated oil with an acid solution, separating and filtering the 30 oil.

19. The process of refining viscous hydrocarbon distillate which comprises acting thereupon with strong sulfuric acid, separating the sour oil, heating it to about 380° 35 F. for eighteen to twenty hours while passing steam therethrough and subsequently filtering the oil.

20. The process of destroying emulsion inducing compounds including sulfo-compounds present in a heavy oil distillate containing the heavy constituents of a 90 to 95% distillate fraction of an oil previously subjected to heavy treatment with sulfuric acid, 40 said distillate having been subsequently subjected to a like treatment with fuming sulfuric acid and being sour in character, comprising heating such sour distillate oil to about 380° F. for 18 to 20 hours while passing steam therethrough, and filtering the oil. 45

ERNEST B. COBB.